

## UNITED STATES PATENT OFFICE

2,213,856

LUBRICATING OIL AND LUBRICATION  
THEREWITHElmer William Cook, New York, N. Y., assignor to  
Tide Water Associated Oil Company, Bayonne,  
N. J., a corporation of DelawareNo Drawing. Application July 6, 1938,  
Serial No. 217,718

10 Claims. (Cl. 252—53)

This invention relates to mineral oil compositions comprising petroleum oils of a viscous or lubricating nature as contrasted with non-viscous hydrocarbons of the character of gasoline or kerosene. It is particularly concerned with mineral oil compositions comprising lubricating and like oils having incorporated therewith small but sufficient amounts of an organic arsenite effective to inhibit or retard deterioration and deterioration 5 effects in service.

The present application is a continuation-in-part of my copending application Serial No. 131,785, filed March 19, 1937, for improvements in Lubricating oil and lubrication therewith; and 15 in one important embodiment the present invention is concerned with lubricants intended for service in the lubrication of internal combustion engines. These now are frequently equipped with bearings comprising or surfaced with cadmium-silver, cadmium-nickel, copper-lead or like alloys having substantially the corrosion susceptibility of the stated alloys. Such harder, higher melting alloys are in certain respects better adapted to the requirements of modern internal 20 combustion engines than the conventional Babbitt metal bearings, in view of greatly increased bearing pressures and the high temperatures which may obtain at bearing surfaces during operation. The mechanical superiority of cadmium-silver and other special alloy bearings is 25 largely offset, however, by a marked susceptibility to corrosion under service conditions by many available lubricating oils—particularly oils which by nature or refining are of the character generally regarded as superior lubricants by conventional criteria (e. g., high viscosity index, substantially or reasonably free from sludge-forming tendencies, etc.).

Under service conditions the presence of cadmium-silver and like alloys appears to catalyze reactions tending toward lubricant degradation. Such alloys likewise seem to be particularly susceptible to corrosion by lubricants which have undergone deterioration in service. It has been 40 suggested that corrosion of bearing metals in internal combustion engines involves a cyclic action or chain of reactions in the course of which the catalytic effect of the bearing metal accelerates oil deterioration and the products of deterioration in turn attack the bearing surfaces with resultant corrosion thereof.

The invention, however, is concerned with retarding lubricant deterioration and deterioration effects without limitative regard to the foregoing 45 or other theory which may be advanced to ex-

plain causes or results. It has been found that organic arsenites including both alkyl and aryl derivatives comprise a class providing compounds effective to inhibit oil deterioration and deterioration effects. According to the invention, service 5 degradation of oils is retarded and the corrosiveness of motor oils to cadmium-silver and like alloys markedly diminished by dissolving in the oil prior to use small but sufficient proportions of an organic arsenite inhibitor. It is, therefore, 10 an object of the invention to improve, and to prepare improved, lubricating oils of petroleum origin by incorporating therein an organic arsenite inhibitor in small but effective proportions. In a special aspect, the invention may be re- 15 garding as encompassing a novel method of lubricating bearings surfaced with an alloy having substantially the corrosion susceptibility of cadmium-silver, cadmium-nickel or copper-lead alloys by applying to the bearing surfaces lubricant 20 comprising mineral hydrocarbon oil normally tending to corrode such alloys and having incorporated therein corrosion-retarding proportions of an organic arsenite inhibitor.

Inhibitors according to the invention are com- 25 pounds conforming to the general formula



30

wherein the R's designate organic radicals such as hydrocarbon residues which may be aryl or alkyl, or may be substituted aryl or alkyl groups. Among the alkyl arsenites, those having from 4 to about 10 carbon atoms in the alkyl residues are 35 presently preferred and the aliphatic chain may be either straight or branched. The preferred aryl arsenite inhibitors according to the invention are the phenyl and cresyl arsenites in view of the greater solubility of these compounds as compared with the higher molecular weight aryl arsenites. The invention also embraces arsenites in which the organic radical is an alicyclic hydrocarbon residue of aliphatic character as in the case of tri-cyclo-hexyl arsenite. The hydrocarbon radicals in both alkyl and aryl arsenites may be substituted at one or more carbon atoms by such groups as alkyl, aryl, aralkyl, alkoxy, amino, hydroxy, and nitro radicals. Inhibitors selected from the defined class need not consist solely of one or another pure organic arsenite, mixtures being effective. This is a beneficial aspect of the invention, since the synthesis of a given arsenite frequently is accompanied by the by-product formation of small amounts of a related compound (e. g. 45 50 55

some tri-ortho cresyl arsenite may be formed in the synthesis of tri-para cresyl arsenite. In such cases it is unnecessary to carry refinement of the reaction product to the point of isolating 5 an absolutely pure compound.

Various methods are described in the literature for the synthesis of organic arsenites. In most cases I have found it convenient to employ the simple reaction of tri-oxide of arsenic ( $As_2O_3$ ) 10 and an appropriate alcohol or hydroxy-aromatic compound with the aid of heat. Water is evolved during the reaction and is continuously removed as steam, heating being continued until all water has been driven off. The reaction mixture then 15 is cooled, anhydrous benzene added, and any residual unreacted tri-oxide of arsenic removed by filtration. The benzene diluent and residual unreacted alcohol are readily removed from the filtrate by distillation under reduced pressure. The 20 organic arsenite product may be refined to desired extent by conventional methods.

Using the foregoing general method of synthesis, tri-phenyl arsenite may be prepared by reacting tri-oxide of arsenic with phenol, the end 25 product being a slightly yellow, viscous liquid having a boiling point of approximately 300° C. at 20-25 mm. mercury. Tri-isoamyl arsenite is produced by using iso-amyl alcohol as the appropriate reagent, the product in this instance being a 30 colorless, mobile liquid boiling at about 150° C. at 10 mm. mercury. To produce tri-cresyl arsenites, an appropriate cresol is used, the product in the case of tri-para cresyl arsenite, for example, being a viscous, yellow liquid. In the case of naphthyl 35 arsenites a suitable naphthol, for example, beta-naphthol, is reacted with tri-oxide of arsenic. Tri-butyl arsenites may be prepared with the aid of butyl or iso-butyl alcohol and colorless liquid products are obtained, the iso compound, for 40 example, boiling at 242° C. under normal atmospheric pressure. Tri-cyclo-hexyl arsenite is produced by the reaction of cyclo-hexyl alcohol with tri-oxide of arsenic; and similarly for other alkyl or aryl arsenites which comprise effective inhibitors according to the invention. 45

The individual effectiveness of organic arsenite inhibitors will vary somewhat as might be expected, some being more effective than others in given proportions. In general it is preferred to 50 use those having greatest inhibitor effectiveness at small concentrations.

As indicated hereinbefore, organic arsenite inhibitors have proved markedly effective in retarding the corrosion of bearing metals by lubricating 55 oils normally corrosive thereto under high temperature service conditions obtaining in internal combustion engines. Concurrent oil deterioration as evidenced by undesirable increases in viscosity, carbon residue, neutralization number and 60 Indiana precipitation number also is retarded in beneficial degree by the use of inhibitors as herein disclosed. Generally, the circumstances giving rise to the need for inhibitors in motor oil service, particularly the problem of bearing corrosion, 65 include high operating temperatures, for example 300° F.-400° F. or even higher in certain localized areas. The present invention provides an adequate over-all improvement in lubricants and in lubrication for such service.

70 The utility of organic arsenite inhibitors extends likewise to lubrication with mineral oils under service conditions involving lower operating temperatures. By way of further illustration may be mentioned in particular the value of such 75 inhibitors in turbine oil service. In such use, the

oil temperature is relatively low, as compared with temperatures encountered in high speed internal combustion engines, but contacted metal surfaces may catalyze acid or sludge formation in the lubricant with eventual emulsification due to the presence of water. Inhibitors according to the invention serve efficiently in retarding oil deterioration under such service conditions. 5

Thus it will be seen that the invention supplies 10 inhibitors of broad utility in mineral oil environment. Mineral oils of lubricating viscosity are definitely improved for a wide range of services by the addition thereto of an organic arsenite inhibitor in small but sufficient proportions to 15 retard oil deterioration and deterioration effects.

The proportion of an organic arsenite inhibitor necessary to accomplish the objects of the present invention is quite small, percentages of the order of 0.05%-0.2% by weight or even less dissolved in 20 mineral lubricating oil exhibiting a marked inhibiting effect. Larger proportions within the limit of solubility for a given arsenite may be used, if desired but the smaller proportions ordinarily are wholly sufficient and, in the interests of economy, preferable. In the illustrative tests reported 25 hereinafter certain specific proportions of inhibitor were used, but stated percentages herein are not intended as a limitation upon the contemplated scope and practice of the invention. The inhibitors may be, and are intended to be, employed in any inhibiting proportion. 30

The tendency of motor oils to corrode bearing 35 metals may be determined by a convenient test which affords a ready method of obtaining a comparative evaluation of motor oils in the laboratory. In this test method a group of bearings, ordinarily including at least one each of several of the newer bearing metal alloys (viz: cadmium-silver, cadmium-nickel and copper-lead) is supported in a chamber in which air may circulate 40 and the bearing surfaces are exposed for a period of 22 hours to a stream of oil sprayed under pressure continuously upon the corrodible area. The oil is maintained at a temperature of approximately 335° F. and the spray is so directed as to 45 disperse the oil over the surfaces of the bearings. Means are provided for recirculating the sprayed oil so that a given quantity is used for a given test, thus simulating service conditions in an engine. The measure of corrosion is taken as the loss in 50 weight of the bearing per unit of exposed corrodible surface. Concurrent oil deterioration is determined by tests on the used oil after a given run.

The test method described above is carried out 55 in the familiar Underwood corrosion apparatus supplied by the Scientific Instrument Company of Detroit, Michigan, in accordance with General Motors specifications.

Results obtained utilizing the foregoing test for 60 comparative evaluation of motor oils with and without an inhibitor according to the invention provide specific illustration of the value and inhibiting effectiveness of triphenyl arsenite. The 65 oil used for the test was an S. A. E. 20 motor oil comprising a blend of well refined paraffinic base stocks and having an A. P. I. gravity of 30.1, Saybolt viscosity at 100° F. of about 300 seconds, Saybolt viscosity at 210° F. of 54 seconds and flash 70 point of 425° F. Inhibitor, when added, was used in an amount of 0.2% by weight based on the oil. During each run cadmium-silver, cadmium-nickel and copper-lead bearings all were present; and comparative losses in weight per square decimeter 75

due to corrosion were observed as follows for the respective bearings:

*Example A*

|    | Bearing             | Oil blank | Oil plus triphenyl arsenite |
|----|---------------------|-----------|-----------------------------|
|    |                     | Grams     | Grams                       |
| 10 | Cadmium-silver..... | 6.6       | 0.1                         |
|    | Cadmium-nickel..... | 5.2       | 0.6                         |
|    | Copper-lead.....    | 0.9       | 0.07                        |

*Example B*

|    | Bearing             | Oil blank | Oil plus tri-p-cresyl arsenite |
|----|---------------------|-----------|--------------------------------|
|    |                     | Grams     | Grams                          |
| 20 | Cadmium-silver..... | 5.1       | 0.6                            |
|    | Cadmium-nickel..... | 9.0       | 1.8                            |
|    | Copper-lead.....    | 3.0       | 0.2                            |

*Example C*

|    | Bearing             | Oil blank | Oil plus tri-iso-amyl arsenite |
|----|---------------------|-----------|--------------------------------|
|    |                     | Grams     | Grams                          |
| 30 | Cadmium-silver..... | 5.1       | No loss.                       |
|    | Cadmium-nickel..... | 9.0       | Do.                            |
|    | Copper-lead.....    | 3.0       | Do.                            |

The used oil tests in Example A were as follows:

|    |                               | Oil blank | Oil plus inhibitor |
|----|-------------------------------|-----------|--------------------|
|    | A. P. I. gravity.....         | 23.1      | 27.0               |
|    | Saybolt vis. @ 100° F.....    | 727       | 470                |
|    | Saybolt vis. @ 210° F.....    | 77        | 64                 |
| 40 | Carbon residue.....           | 3.60      | 1.85               |
|    | Neutralization No.....        | 5.65      | 3.41               |
|    | Indiana precipitation No..... | 13.0      | 11.0               |

In Example B the used oils had the following comparative tests:

|    |                               | Oil blank | Oil plus inhibitor |
|----|-------------------------------|-----------|--------------------|
|    | A. P. I. gravity.....         | 19.1      | 26.1               |
|    | Saybolt vis. @ 100° F.....    | 3266      | 528                |
|    | Saybolt vis. @ 210° F.....    | 151       | 69                 |
|    | Carbon residue.....           | 3.72      | 2.30               |
| 50 | Neutralization No.....        | 12.0      | 3.36               |
|    | Indiana precipitation No..... | 23        | 7                  |

The used oils in Example C had the following tests:

|    |                               | Oil blank | Oil plus inhibitor |
|----|-------------------------------|-----------|--------------------|
|    | A. P. I. gravity.....         | 19.1      | 28.4               |
|    | Saybolt vis. @ 100° F.....    | 3266      | 387                |
|    | Saybolt vis. @ 210° F.....    | 151       | 60                 |
|    | Carbon residue.....           | 3.72      | 1.22               |
| 60 | Neutralization No.....        | 12.0      | 1.18               |
|    | Indiana precipitation No..... | 23        | 6                  |

It will be clear from all of the foregoing evidence that not only does the presence of an organic arsenite inhibitor effect a marked retardation of bearing corrosion, but that the presence 70 of the inhibitor likewise reduces substantially the concurrent deterioration of the oil.

Actual tests in an engine equipped with alternate cadmium-silver and copper-lead bearings, and operated under conditions far more severe 75 than those ordinarily encountered under most

service conditions, gave ample confirmation of the results obtained in the laboratory tests reported above. It will be clear, therefore, that the invention provides efficiently improved lubrication for internal combustion engines, particularly those equipped with bearings of the cadmium-silver type. Ordinarily the oil selected for use, in applying the lubricating method of the invention to its intended service, will be of a character generally regarded as of superior grade and refining, i. e., of the low sludge forming or relatively sludge-resistant type as evaluated by conventional tests such as the Indiana oxidation test. Thus, the invention finds particular utility in making possible beneficial use of such oils in internal combustion service by avoiding deleterious consequences otherwise encountered when no preventive measures are taken against the corrosive deterioration of bearing metal alloys as hereinbefore referred to.

By another test method, which has proved of particular convenience in, although not limited to, the evaluation of oils intended for such service as the lubrication of steam turbines, the broad range of effectiveness characterizing organic arsenite inhibitors may be further demonstrated. In this test the deterioration of mineral lubricating oil under relatively low temperature service conditions is accelerated in marked degree, thereby making it possible to compare the relative tendencies toward deterioration of various oils with and without inhibitors. A measured quantity of oil and water (ordinarily 300 cc. of oil and 30 cc. of distilled water) is placed in a small closed brass chamber or capsule, in which an air pressure of 50#/sq. in. is maintained, and subjected to violent agitation for a test period of 150 hours with the chamber immersed during the test period in a steam bath maintained at approximately 212° F. Air in the chamber is 40 changed at 24 hour intervals to insure a sufficiency of oxygen throughout the test period. The neutralization number (milligrams KOH equivalent per gram of oil) of the oil layer at the end of the test period is taken as the measure of deterioration.

*Example D*

The oil used was a turbine oil produced from an East Texas crude, which oil had been refined by solvent extraction with liquid sulfur dioxide and had a viscosity at 100° F. of approximately 150 Saybolt seconds, an iodine number of about 10, and a color of about 1 A. S. T. M. The following comparative results were obtained:

| Inhibitor                                 | Neutralization No. of oil layer after test |
|-------------------------------------------|--------------------------------------------|
| None (average value of several runs)..... | 0.21                                       |
| 0.05% tri-phenyl arsenite.....            | 0.08                                       |

The data tabulated above show clearly the effectiveness of an inhibitor according to the invention in retarding the deterioration of a well refined medium viscosity mineral oil of a character adapted to steam turbine lubrication service.

It will be understood, of course, that all of the foregoing examples are given by way of illustration and not by way of limitation; the use of an inhibitor according to the invention, in other than the specific proportions mentioned and in other than the specifically designated oils, being within the contemplated scope thereof.

I claim:

1. Method of lubricating bearing surfaces, at least one of which comprises an alloy having substantially the corrosion susceptibility of cadmium-silver, cadmium-nickel and copper-lead alloys, which comprises applying to the bearing surfaces lubricant having incorporated therein a sufficiently oil-soluble alkyl arsenite in corrosion inhibiting proportions.
  10. Method of lubricating bearing surfaces, at least one of which comprises an alloy having substantially the corrosion susceptibility of cadmium-silver, cadmium-nickel and copper-lead alloys, which comprises applying to the bearing surfaces lubricant having incorporated therein corrosion inhibiting proportions of a tri-amyl arsenite.
  20. Method of lubricating bearing surfaces, at least one of which comprises an alloy having substantially the corrosion susceptibility of cadmium-silver, cadmium-nickel and copper-lead alloys, which comprises applying to the bearing surfaces lubricant having incorporated therein corrosion inhibiting proportions of a tri-butyl arsenite.
  30. Method of lubricating bearing surfaces, at least one of which comprises an alloy having substantially the corrosion susceptibility of cadmium-silver, cadmium-nickel and copper-lead alloys, which comprises applying to the bearing surfaces lubricant having incorporated therein corrosion inhibiting proportions of tri-iso-amyl arsenite.
  35. Method of lubricating bearing surfaces, at least one of which comprises an alloy having substantially the corrosion susceptibility of cadmium-silver, cadmium-nickel and copper-lead
- alloys, which comprises applying to the bearing surfaces lubricant having incorporated therein corrosion inhibiting proportions of tri-iso-butyl arsenite.
6. Mineral oil composition suitable for internal combustion engine and steam turbine lubrication comprising a relatively heavy, viscous lubricating oil normally subject to deterioration in service containing an alkyl arsenite in a small but sufficient amount to inhibit said deterioration.
  10. Mineral oil composition suitable for internal combustion engine and steam turbine lubrication comprising a relatively heavy, viscous lubricating oil normally subject to deterioration in service containing a tri-amyl arsenite in a small but sufficient amount to inhibit said deterioration.
  15. Mineral oil composition suitable for internal combustion engine and steam turbine lubrication comprising a relatively heavy, viscous lubricating oil normally subject to deterioration in service containing a tri-butyl arsenite in a small but sufficient amount to inhibit said deterioration.
  20. Mineral oil composition suitable for internal combustion engine and steam turbine lubrication comprising a relatively heavy, viscous lubricating oil normally subject to deterioration in service containing a tri-iso-amyl arsenite in a small but sufficient amount to inhibit said deterioration.
  25. Mineral oil composition suitable for internal combustion engine and steam turbine lubrication comprising a relatively heavy, viscous lubricating oil normally subject to deterioration in service containing tri-iso-amyl arsenite in a small but sufficient amount to inhibit said deterioration.
  30. Mineral oil composition suitable for internal combustion engine and steam turbine lubrication comprising a relatively heavy, viscous lubricating oil normally subject to deterioration in service containing tri-iso-butyl arsenite in a small but sufficient amount to inhibit said deterioration.
  35. Mineral oil composition suitable for internal combustion engine and steam turbine lubrication comprising a relatively heavy, viscous lubricating oil normally subject to deterioration in service containing tri-iso-butyl arsenite in a small but sufficient amount to inhibit said deterioration.

ELMER WILLIAM COOK.